

## UNITED STATES PATENT OFFICE

HARRY J. JOHN, OF WASHINGTON, PENNSYLVANIA, ASSIGNOR, BY MESNE ASSIGNMENTS, TO NORMAN A. EMERY, OF YOUNGSTOWN, OHIO

## PICKLING COMPOSITION

No Drawing.

Application filed April 2, 1927. Serial No. 180,627.

This invention relates to pickling processes such as are used in the removal of scale from steels and has for its object to reduce the time of pickling, and to make it safer and cheaper.

5 In pickling steel it is common to heat the acid solution to expedite the chemical action. If this chemical action is further hastened by increase in acid strength it is unsatisfactory because the stronger acid not only attacks the scale but also the body of metal. If the temperature of the bath is raised too high, evaporation causes waste in acid. Another source of trouble is the release of bubbles of hydrogen, which rise 10 and pass out of the bath carrying particles of acid spray to the injury of exposed metal parts of the building and the workmen. Under this invention these disadvantages are greatly reduced as is also the time of 15 pickling.

According to this invention a substance like palladium sponge having a strong affinity for hydrogen is suspended in the bath. A salt is also added to the bath capable of 20 being acted on to renew the acid and forming a material which inhibits the action of the acid on and protects the body of metal. To lessen loss of acid through vaporization, and assist in acid renewal, a floatable solid 25 or vegetable matter like sawdust or spent tanbark is spread over the surface to cover the bath.

The usual treatment tank and crate for the material being pickled is used.

30 For treatment of a low carbon copper nickel steel a 2% to 20% bath of mixed hydrochloric and nitric acids is used, two parts of hydrochloric to one of nitric being found desirable. About 2% to 5% by weight of sodium chloride (rock salt) is added and dissolved. Throughout the bath is distributed a material having an affinity for hydrogen. This is preferably palladium sponge attached to various portions of the crate containing the material to be pickled, as for example by means of bronze wire, and about 1 lb. of the palladium sponge for each 2,000 gallons of the bath has been found satisfactory. After the crated material has been 45 placed in the bath a quantity of floatable,

solid material like sawdust, spent tanbark, or quebracho bark is spread over to cover substantially the entire surface of the bath and lessen vaporization. The bath is preferably heated by live steam to a temperature 55 of 170° to 180° F. On completion of the pickling operation the material is taken out free from scale and immersed in warm rinse water, then in a hot soap solution or otherwise as is customary, to entirely remove the acid from the material.

The palladium sponge has a strong affinity for hydrogen and is capable of absorbing such a large quantity of hydrogen that the sponge in usual practice would not become 65 saturated until in use about a week. Evidence that the palladium sponge has become saturated is seen in the emission of hydrogen from the bath. When saturated the palladium sponge is removed, placed in a crucible and heated to about 800° C. or as low as 500° C. if a vacuum is used, with the result that the hydrogen is burned out, but no oxidation of the sponge occurs at these temperatures. When the hydrogen has been 75 burned out the palladium sponge is ready to be used over again in the bath.

The acid used for the bath depends on the kind of materials treated. Where tungsten or chrome steels are treated it has been found desirable to use a mixture of hydrochloric and sulphuric acids. But with a copper or nickel steel the use of hydrochloric and nitric acids is preferred. Commercial sulphuric or hydrochloric acid contains certain impurities 80 such as arsenic and antimony which ordinarily have an affinity for the nascent hydrogen, with the result that hydrogen compounds of these materials are precipitated on the metal surfaces in pin spots, which are difficult to coat with tin, zinc, and the like. The palladium sponge having a stronger affinity for hydrogen than the acid impurities, there is no union and precipitation of these impurities on the metal surface with the result that this surface is cleaner and better adapted for coating. The acid strength depends on the alloy used and when treating a low carbon copper nickel steel alloy it has been found 85 that the acid strength may be increased to 90 95 100

10% to 20% to expedite the pickling. The strength of acid also depends on the amount of scale and the kind of acid used.

The precise nature of what takes place in this invention is uncertain, for the reactions are complex. The several features of this invention contribute to the production of better pickling results than would be expected from their separate use in old processes. The 10 sodium chloride is acted upon by the nitric acid to renew the acid and form sodium nitrate and hydrochloric acid, either directly or by the union of nascent hydrogen and chlorine. It is thought the sawdust floating on 15 the surface, beside reducing vaporization, facilitates acid renewal by precluding the escape of chlorine, any hydrogen not absorbed, and any hydrochloric acid gas coming off from the heated bath. The sawdust 20 also functions to absorb any oil or grease on the bath and thus prevent such from getting on the metal surface. The sodium nitrate formed functions as an inhibitor to lessen acid action on the metal body without unduly 25 reducing its activity on scale. It is thought that nitric acid, being an oxidizing agent, oxidizes some of the lower oxide scale to higher oxides to render them more susceptible of attack by acid. By reason of the renewal 30 of the acid, a weaker initial acid strength is capable of accomplishing greater results than would the corresponding acid strength which is not renewed. It is thought that palladium facilitates action of the acid on the metal 35 where, as here, the solution is dilute. The sodium chloride acts as an inhibitor during the formation of the sodium nitrate.

What is claimed is:

1. An acid pickling solution comprising 40 hydrochloric acid, sodium chloride, another mineral acid capable of acting on sodium chloride to renew the strength of hydrochloric acid, and particles of solid material floating on the surface of the bath to lessen 45 the escape of gas, thereby enhancing the strength of the hydrochloric acid.
2. An acid pickling bath containing palladium sponge and sawdust spread over to substantially cover the surface of the bath.
- 50 3. An acid pickling solution containing palladium.
4. An acid pickling solution containing palladium sponge suspended therein.
5. A pickling solution containing a mixture 55 of hydrochloric and nitric acids and sodium chloride.
6. A pickling solution containing a 2% to 20% mixture of hydrochloric and nitric acids with roughly about 2% to 5% of sodium chloride, there being a larger amount of nitric than hydrochloric acid.
- 60 7. A pickling solution containing about two parts of hydrochloric to one part of nitric acids in the presence of sodium chloride.
- 65 8. A pickling solution containing a mix-

ture of hydrochloric acid and a large amount of nitric acid, sodium chloride, and palladium sponge.

9. An acid pickling solution having floating particles of solid substance substantially 70 covering the surface of the bath, and containing within the bath distributed, palladium sponge.

10. A pickling solution containing sodium chloride, hydrochloric acid, and another acid 75 which reacts with sodium chloride to renew the hydrochloric acid and form an inhibitor.

11. A pickling solution containing sodium chloride, hydrochloric acid and another acid which reacts with sodium chloride and 80 is an oxidizing agent for scale.

In testimony whereof I have hereunto set my hand this 31 day of March, 1927.

HARRY J. JOHN.